# EUROPEAN PATENT SPECIFICATION

(11) **EP 1 723 223 B1**
(45) Date of publication and mention of the grant of the patent: **29.10.2008**
(21) Application number: 05716869.2
(22) Date of filing: 02.03.2005
(51) Int. Cl.: C11D 3/42, C09B 23/14

(54) **PROCESS FOR THE PREPARATION OF BRIGHTENER PIGMENTS**
VERFAHREN ZUR HERSTELLUNG VON AUFHELLENDEN PIGMENTEN
PROCEDE POUR LA PREPARATION D'UN PIGMENT OPTIQUE FLUORESCENT

(30) Priority: 12.03.2004 EP 04101017
(43) Date of publication of application: 22.11.2006
(73) Proprietor: Ciba Holding Inc., 4057 Basel (CH)
(72) Inventor: HOCHBERG, Robert, 79249 Merzhausen (DE); BECHERER, Oliver, 79739 Schwörstadt (DE); MERKLE, Gerhard, 79102 Freiburg (DE)
(74) Representative: Bohest AG
(86) International application number: PCT/EP2005/050903
(87) International publication number: WO 2005/090545

(56) References cited:
- EP-A- 0 900 783
- WO-A-00/58432
- WO-A-03/104560
- DE-A- 4 401 471

## Description

The present invention relates to a process for the preparation of a brightener pigment comprising
(a) a water-insoluble urea-formaldehyde resin having a water content of more than or equal to 50% by weight, and
(b) a water-soluble fluorescent whitening agent,
which process comprises
adding together (a), (b) and an inorganic salt, the amount of the inorganic salt being sufficient to effect deposition of the water-soluble fluorescent whitening agent (b) on the water-insoluble urea-formaldehyde resin (a).

Preferably, there is used in accordance with the invention a water-insoluble urea-formaldehyde resin of which the molar ratio of urea to formaldehyde is from 1:1.3 to 2 moles.

The urea-formaldehyde resin is also distinguished by a small particle diameter of from 0.01 to 100 µm, especially 0.01 to 50 µm. Highly preferred is a particle diameter of from 0.01 to 20 µm, especially 0.01 to 10 µm.

In general, the BET specific surface area of the urea-formaldehyde resin is of from 2 to 200 m²/g, especially 5 to 120 m²/g. Highly preferred is a BET specific surface area of from 5 to 50 m²/g.

The BET specific surface area of the preferred water-insoluble urea-formaldehyde resins is ascertained according to the Brunauer, Emmett and Teller method [cf. J.Am.Chem.Soc. 60, 309-319 (1938), Chemie-Ing.Techn. 32, 349-354 (1960) and 35, 568-589 (1963)] according to DIN 66132.

The water-insoluble urea-formaldehyde resins, which correspond to component (a), and the preparation of those polymers, are known, for example, from A. Renner: Makromolekulare Chemie 149, 1-27 (1971). Brightener pigments used in detergents and cleaners, and processes for the production thereof are known from EP0900783-A1 and WO00/58432-A1.

The component (a) compounds are prepared by reacting formaldehyde with urea in aqueous solution in the above-described ratios. The reaction is carried out preferably in two steps. In the first reaction step, urea is reacted with formaldehyde according to a customary condensation mechanism, resulting in a low-molecular-weight, water-soluble pre-condensate. In the second reaction step, an acid catalyst can be used in order to accelerate the reaction and for crosslinking, an insoluble, finely divided solid being obtained.

The water content of the reaction solution should never be lower than the total weight of the reactants present in the reaction mixture, and should preferably be higher than the total weight of all the other components in the reaction mixture during the precipitation of the insoluble polymer particles.

The reaction temperature in the first reaction step is usually in the range from 20 to 100°C. The pH can be adjusted to from 6 to 9 by the addition of a strong, aqueous, inorganic base, such as, for example, sodium hydroxide solution.

Advantageously, the preparation of the pre-condensate can be carried out in the presence of a surfactant. The surfactant is used, for example, in amounts of from 0.5 to 5 % by weight, based on the total weight of the urea and formaldehyde. Ionic surfactants cause an increase in the specific surface area of the urea-formaldehyde polymer product, whereas non-ionic surfactants have the opposite effect.

Advantageously, the first reaction step is carried out in the presence of a macromolecular water-soluble protective colloid having polyelectrolytic properties. Examples of such protective colloids include gelatin, tragacanth, agar and polyvinylpyrrolidone, especially methacrylic acid. The amount of protective colloid used can be within a range of, for example, from 0.5 to 5 % by weight, based on the total weight of urea and formaldehyde. Neither polyvinylpyrrolidone nor polymethacrylic acid causes an increase in the specific surface area of the water-insoluble urea-formaldehyde resin.

One of the most important conditions for the successful preparation of non-meltable, insoluble and finely divided urea-formaldehyde polymers that meet the qualitative requirements of the brightener pigments in accordance with the invention is the use in the second reaction step of a suitable catalyst for gel formation. Suitable catalysts include, for example, relatively strong inorganic and/or organic acids, such as, for example, sulfuric acid, sulfurous acid, sulfamic acid, phosphoric acid, hydrochloric acid, chloroacetic acid, maleic acid or maleic anhydride. Generally, such gel-formation catalysts should have an ionisation constant in excess of 10⁻⁴. Sulfuric acid and its acidic ammonium or amine salts, and also ammonium sulfate, methylamine hydrogen sulfate and ethanolamine hydrogen sulfate, are preferred. The acids are generally used in the form of 1 to 15 % by weight aqueous solutions. As a rough guide, from 20 to 100 mmoles of a crosslinking catalyst are used per mole of urea added. This causes a reduction in the pH of the reaction mixture to from 1 to 3.0 in the second reaction step during the formation of the polymer.

When sulfamic acid is used, water-insoluble urea-formaldehyde resins having a relatively high specific surface area are generally obtained, the other acids of those mentioned above, especially sulfuric acid and its ammonium or amine salts, having the opposite effect.

The reaction temperatures in the second, resin-forming reaction step usually reach from 20 to 100°C. Large differences in temperature in the reaction mixture should be avoided during the addition of the catalyst. It is therefore desirable to heat the aqueous catalyst solution to the temperature of the reaction mixture before it is added to that mixture. Generally, a white gel is obtained after only from 15 to 30 seconds. The crosslinking reaction is usually finished after a reaction time of from 30 minutes to 3 hours.

The insoluble polymer is obtained in the form of a white gel and can be comminuted mechanically, treated with a desired amount of water, adjusted with alkali or ammonium hydroxide to a pH of from 6 to 9, and then isolated from the aqueous phase, for example by filtration, centrifugation or concentration by evaporation. If desired, drying can be carried out e.g. by spray-drying or convection-drying, to prepare corresponding polymers having a specified water content.

The gel obtained is then worked up in customary manner, for example by allowing the reaction to proceed to completion, neutralising, and then filtering, washing, drying and, if desired, grinding to obtain a suitable particle size.

The water content of the water-insoluble urea-formaldehyde resin is preferably 50 to 90% by weight, especially 60 to 90% by weight. Highly preferred is a water content of 60 to 80% by weight. An example of such resins is Pergopak^{®} HP. In the following, the weight of the urea-formaldehyde resin is to be understood to include the weight of water.

The ratio by weight of fluorescent whitening agent to urea-formaldehyde resin is typically 1:1000 to 1:10, especially 1:500 to 1:10. Highly preferred is a weight ratio of 1:250 to 1:50, especially 1:200 to 1:100.

Typical concentrations of the urea-formaldehyde resins used in the preparation process are 1 to 600 g/l, especially 10 to 600 g/l. Highly preferred concentrations of the urea-formaldehyde resins are 100 to 600 g/l, especially 200 to 600 g/l.

Preferred fluorescent whitening agents corresponding to component (b) that can be used in accordance with the invention correspond to formula in which formulae
- each R₁: is independently from each other a radical of formula -NH₂; -O-C₁-C₄alkyl; -O-aryl; -NH-C₁-C₄alkyl; -N(C₁-C₄alkyl)₂; -N(C₁-C₄alkyl)(C₁-C₄hydroxyalkyl); -N(C₁-C₄hydroxyalkyl)₂; -NH-aryl; morpholino or -S-C₁-C₄alkyl(aryl);
- each R₂: is independently from each other hydrogen; an unsubstituted or substituted alkyl or aryl group; a radical of formula -OH; -NH₂; -N(CH₂CH₂OH)₂; -N[CH₂CH(OH)CH₃]₂; -NH-R₄; -N(R₄)₂; -OR₄; -Cl; , -O-C₁-C₄alkyl; -O-aryl; -NH-C₁-C₄alkyl; -N(C₁-C₄alkyl)₂; -N(C₁-C₄alkyl)(C₁-C₄hydroxyalkyl); -N(C₁-C₄hydroxyalkyl)₂; -NH-aryl, or -S-C₁-C₄alkyl(aryl);
- R₃: is an unsubstituted or substituted alkyl or aryl group;
- each R₄: is independently from each other M, or an unsubstituted or substituted alkyl or aryl group;
- R₅: is hydrogen; an unsubstituted or substituted alkyl or aryl group; or -NR₇R₈, wherein R₇ and R₈ are each independently of the other hydrogen or an unsubstituted or substituted alkyl or aryl group, or R₇ and R₈ together with the nitrogen atom linking them form a heterocyclic radical, especially a morpholino or piperidino radical;
- R₆: is hydrogen, or an unsubstituted or substituted alkyl or aryl group;
- R₉ and R₁₀: are each independently of the other hydrogen, C₁-C₄alkyl, phenyl or a radical of formula
- R₁₁: is hydrogen, -Cl or SO₃M;
- each R₁₂: is independently from each other -CN; -SO₃M; -S(C₁-C₄alkyl)₂ or -S(aryl)₂;
- each R₁₃: is independently from each other hydrogen; -SO₃M; -O-C₁-C₄alkyl; -CN; -Cl; COO-C₁-C₄alkyl or -CON(C₁-C₄alkyl)₂;
- each R₁₄: is independently from each other hydrogen; -C₁-C₄alkyl; -Cl or -SO₃M;
- R₁₅ and R₁₆: are each independently of the other hydrogen, C₁-C₄alkyl; -SO₃M; -Cl or -O-C₁-C₄alkyl;
- each R₁₇: is independently of the other hydrogen or C₁-C₄alkyl;
- R₁₈: is hydrogen, C₁-C₄alkyl; -CN; -Cl; -COO-C₁-C₄alkyl; -CON(C₁-C₄alkyl)₂; aryl or -O-aryl;
- B: is
- M: is hydrogen; sodium; potassium; calcium; magnesium; ammonium; mono-, di-, tri- or tetra-C₁-C₄alkylammonium; mono-, di- or tri-C₁-C₄ hydroxyalkylammonium; or ammonium di- or tri-substituted by a mixture of C₁-C₄alkyl and C₁-C₄hydroxyalkyl groups; and
- n₁, n₂ and n₃: are each independently of the others 0 or 1.

R₂, R₃, R₄, R₅, R₆, R₇ and R₈ representing (unsubstituted or) substituted alkyl are each C₁-C₁₂alkyl, preferably C₁-C₄alkyl. The alkyl groups may be branched or unbranched and may be unsubstituted or substituted by halogen, e.g. fluorine, chlorine or bromine, by C₁-C₄alkoxy, e.g. methoxy or ethoxy, by phenyl or carboxyl, by C₁-C₄alkoxycarbonyl, e.g. acetyl, by mono- or di-C₁-C₄alkylamino or by -SO₃M.

R₂, R₃, R₄, R₅, R₆, R₇ and R₈ representing (unsubstituted or) substituted aryl are each preferably a phenyl or naphthyl group that may be unsubstituted or substituted by C₁-C₄alkyl, e.g. methyl, ethyl, propyl, isopropyl, butyl, isobutyl, sec-butyl or tert-butyl, by C₁-C₄alkoxy, e.g. methoxy, ethoxy, propoxy, isopropoxy, butoxy, isobutoxy, sec-butoxy or tert-butoxy, by halogen, e.g. fluorine, chlorine or bromine, by C₂-C₅alkanoylamino, e.g. acetylamino, propionylamino or butyrylamino, by nitro, by sulfo or by di-C₁-C₄alkylated amino.

The compounds of formula (1) are used preferably in neutral form, that is to say: M is preferably a cation of an alkali metal, especially sodium, or is an amine.

The fluorescent whitening agents that can be used advantageously in the present invention are listed by way of example in the following Table 1:

| Table 1: | |
|---|---|
| Compound of formula | |
| (9) | |
| (10) | |
| (11) | |
| (12) | |
| (13) | |
| (14) | |
| (15) | |
| (16) | |
| (17) | |
| (18) | |
| (19) | |
| (20) | |
| (21) | |
| (22) | |
| (23) | |
| (24) | |
| (25) | |
| (26) | |

The fluorescent whitening agents corresponding to component (b) are employed preferably in amounts of from 0.001 to 10 % by weight, especially from 0.1 to 10 % by weight, and more especially from 0.1 to 5 % by weight, based on the total amount of urea-formaldehyde resin. Highly preferred is an amount of 0.5 to 5 % by weight. The fluorescent whitening agents can be added to the urea-formaldehyde resin in the form of individual compounds or in the form of mixtures of several individual compounds.

It is preferred for the process of the present invention to add the fluorescent whitening agent in the form of an aqueous solution. For such solutions an amount of 0.01 to 20 % by weight of the fluorescent whitening agent, especially 0.1 to 10 % by weight, is preferred. Highly preferred is an amount of 0.5 to 10 % by weight.

Due to the use of an inorganic salt the fluorescent whitening agent can effectively be deposited on the urea-formaldehyde resin. This also enables the preparation of brightener pigments having high concentrations of fluorescent whitening agents.

Preferred inorganic salts are alkali or earth alkali salts, especially chlorides or sulfates. Examples of such salts are sodium chloride, sodium sulfate and calcium chloride, especially sodium sulfate and calcium chloride.

The ratio by weight of inorganic salts to urea-formaldehyde resin is typically 1:500 to 1:1, especially 1:200 to 1:1. Highly preferred is a weight ratio of 1:50 to 1:1, especially 1:20 to 1:1.

Typical concentrations of the inorganic salts used in the preparation process are 1 to 200 g/l. Highly preferred concentrations of the inorganic salts are 10 to 200 g/l, especially 10 to 100 g/l.

The process is usually carried out in aqueous medium. According to a preferred embodiment of the present invention an aqueous suspension or solution is prepared, comprising the fluorescent whitening agent and the urea-formaldhyde resin, and an inorganic salt is added. It is preferred that the addition of the inorganic salt is carried out at elevated temperature, like 30 to 90°C, especially 40 to 90°C. Highly preferred are temperatures of 50 to 90°C, especially 60 to 90°C.

Preferably, the water-soluble fluorescent whitening agent is added before, during or after gelation. Usually, the procedure comprises dispersing the urea-formaldehyde resin in hot water with a vigorous stirring action. If desired, the pH is adjusted to <10 using an aqueous alkali metal hydroxide solution and the water-soluble fluorescent whitening agent is added thereto. However, in general no adjustment of the pH is required. The batch is further stirred for some time and cooled. According to a less preferred variant the pH can be adjusted to <3 using a strong acid, especially sulfuric acid. A viscous suspension is obtained which is isolated by customary methods, such as filtration. If desired, the brightener pigment obtained can be further processed by drying and, optionally, by grinding.

According to a preferred embodiment of the present invention the brightener pigment is isolated, for example by filtration, and no separate drying or milling step is carried out. It is to be noted that the brightener pigments obtained according to the process of the present invention can be used without drying or grinding.

In a further embodiment, the brightener pigment may be subjected to a surface treatment. For that purpose, an emulsion of long-chain alcohols or derivatives thereof, of derivatives of ethylene oxide-alcohols, of paraffin waxes, or of hydrogenated natural or synthetic resins, etc., and especially a dodecanol emulsion, is added to the viscous urea-formaldehyde resin/whitening agent suspension. The batch is stirred for a further 10 to 15 minutes at elevated temperature. After cooling, the batch is filtered and, if desired, can be further processed as given above, yielding a surface-treated formaldehyde resin/whitening agent suspension. However, if desired, the extra step of surface treatment can be omitted.

Dazzlingly white organic brightener pigments are obtained which have a very low content of free formaldehyde (typically less than 0.1% DIN 58187) in which the fluorescent whitening agent has been incorporated or adsorbed. Such products are solid, colloidal particles. Particles of lower diameter can agglomerate to form pigment particles having an average diameter of from, for example, 3 to 20 µm.

Another object of the present invention are additives in the form of a brightener pigment comprising
a) a water-insoluble urea-formaldehyde resin having a water content of more than or equal to 50% by weight, and
(b) a water-soluble fluorescent whitening agent.

As to these additives the definitions and preferences given above apply.

The fluoresecently brightened pigments prepared in that manner are excellently suitable for improving the degree of whiteness (improvement in appearance) of commerically available detergents and cleansers, of compounds thereof, and of individual raw materials.

The brightener pigment used in accordance with the invention is usually incorporated into the detergents or cleansers by first suspending the brightener pigment in water, with stirring, and then adding the detergent or cleanser in question to the resulting suspension with the further addition of water. A creamy slurry is obtained, which is then dried and sieved to yield a detergent or cleanser having a particle size of approximately from > 0.3 to 1 mm.

In a further embodiment, the fluoroscently brightened detergent or cleanser compounds thereof and individual raw materials are prepared by simply dusting with the brightener pigment in powder form. For that purpose from 0.5 to 20%, typically from 1 to 10%, of brightener pigment based on the component to be whitened is dry-mixed until the particles have been coated with the pigment.

Suitable compositions that can be treated in accordance with the invention with the brightener pigment comprising components (a) and (b) are detergents or cleansers in the form of powder or granules. Such formulations may be particulate detergents composed of one or more granular components in which at least one granular component is acted upon by the brightener pigment.

There come into consideration preferably formulations in granular form that have a high bulk density. In addition to the brightener pigment, the detergent may comprise further ingredients, e.g. surfactants, inorganic and organic builder substances, bleaching agents, substances that have a positive effect on the ability to wash out oil and grease, greying inhibitors, if desired substances that improve the solubility and the rate of dissolution of the individual granular components and/or of the entire formulations, fabric-softening substances, colorants and perfumes, and also alkaline and/or neutral salts in the form of their sodium and/or potassium salts.

In addition, washing-active or cleaning-active shaped forms, for example detergent tablets, dishwashing agent tablets, stain-removing salt tablets or water-softening tablets, can be provided in accordance with the invention.

The washing-active or cleaning-active shaped forms are especially cylindrical shapes or tablets that can be used as detergents, dishwashing agents, or bleaching agents (stain-removing salts), but can also be used as pretreatment agents, for example as water softeners or bleaching agents. A distinction is drawn between homogeneous (homogeneously distributed ingredients) and heterogeneous (heterogenously distributed ingredients) shaped forms, which have as a special feature a disintegrator, such as, for example, starch, a starch derivative, cellulose or a cellulose derivative, which brings about the disintegration of the washing-active or cleaning-active shaped form. It is possible, in particular, for the degree of whiteness of such a disintegrator to be excellently improved by the brightener pigments used in accordance with the invention.

The so-treated detergent is distinguished by a very high degree of whiteness, which is substantially higher than that achieved by the discrete addition of organic white pigment and fluorescent whitening agent.

The following Examples illustrate the invention, without the invention being limited thereto.

### Example 1

465 g demineralized water and 375 g of a commercially available urea formaldehyde condensation polymer (Pergopak HP) are filled into a 1.5 I vessel and heated to 65-70°C. After the addition of 2.5 g of the compound of formula (101) the suspension is stirred for 20 minutes at 65-70°C. Subsequently 48 g of sodium chloride are added and the mixture is stirred for another 30 minutes. To this suspension a warm emulsion (70°C) is added that has been prepared separately from 1.2 g 1,2-dodecandiol and 240 g demineralized water. The mixture is stirred for 30 minutes, cooled to 35°C and filtered. 452 g of a white wet cake are obtained.

### Example 2

465 g demineralized water and 375 g of a commercially available urea formaldehyde condensation polymer (Pergopak HP) are filled into a 1.5 I vessel and heated to 65-70°C. After the addition of 2.5 g of the compound of formula (101) the suspension is stirred for 20 minutes at 65-70°C. Subsequently 48 g of sodium chloride are added and the mixture is stirred for another 30 minutes. Then the mixture is cooled to 35-38°C by addition of 290 g crushed ice and filtered. 458 g of a white wet cake are obtained.

### Example 3

465 g demineralized water and 375 g of a commercially available urea formaldehyde condensation polymer (Pergopak HP) are filled into a 1.5 I vessel and heated to 65-70°C. After the addition of 2.5 g of the compound of formula (101) the suspension is stirred for 20 minutes at 65-70°C. Subsequently 48 g of sodium sulfate are added and the mixture is stirred for another 30 minutes. To this suspension a warm emulsion (70°C) is added that has been prepared separately from 1.2 g 1,2-dodecandiol and 240 g demineralized water. The mixture is stirred for 30 minutes, cooled to 35°C and filtered. 449 g of a white wet cake are obtained.

### Example 4

465 g demineralized water and 375 g of a commercially available urea formaldehyde condensation polymer (Pergopak HP) are filled into a 1.5 I vessel and heated to 65-70°C. After the addition of 2.5 g of the compound of formula (101) the suspension is stirred for 20 minutes at 65-70°C. Subsequently 48 g of sodium sulfate are added and the mixture is stirred for another 30 minutes. Then the mixture is cooled to 35-38°C by addition of 290 g crushed ice and filtered. 445 g of a white wet cake are obtained.

### Example 5

465 g demineralized water and 375 g of a commercially available urea formaldehyde condensation polymer (Pergopak HP) are filled into a 1.5 I vessel and heated to 65-70°C. After the addition of 2.5 g of the compound of formula (101) the suspension is stirred for 20 minutes at 65-70°C. Subsequently 3 g of calcium chloride x 2 H₂O are added and the mixture is stirred for another 30 minutes. To this suspension a warm emulsion (70°C) is added that has been prepared separately from 1.2 g 1,2-dodecandiol and 240 g demineralized water. The mixture is stirred for 30 minutes, cooled to 35°C and filtered. 403 g of a white wet cake are obtained.

### Example 6

465 g demineralized water and 375 g of a commercially available urea formaldehyde condensation polymer (Pergopak HP) are filled into a 1.5 I vessel and heated to 65-70°C.

After the addition of 2.5 g of the compound of formula (101) the suspension is stirred for 20 minutes at 65-70°C. Subsequently 3 g calcium chloride x 2 H₂O are added and the mixture is stirred for another 30 minutes. Then the mixture is cooled to 35-38°C by addition of 290 g crushed ice and filtered. 396 g of a white wet cake are obtained.

## Claims

1. A process for the preparation of a brightener pigment comprising
(a) a water-insoluble urea-formaldehyde resin having a water content of more than or equal to 50% by weight, and
(b) a water-soluble fluorescent whitening agent,
which process comprises
adding together (a), (b) and an inorganic salt, the amount of the inorganic salt being sufficient to effect deposition of the water-soluble fluororescent whitening agent (b) on the water-insoluble urea-formaldehyde resin (a).

2. A process according to claim 1, wherein the water content of the water-insoluble urea-formaldehyde resin is 50 to 90% by weight.

3. A process according to claim 1, wherein the water content of the water-insoluble urea-formaldehyde resin is 60 to 90% by weight.

4. A process according to any one of claims 1 to 3, wherein the water-insoluble urea-formaldehyde resin has a molar ratio of urea to formaldehyde of from 1:1.3 to 2 moles, a particle diameter of from 0.01 to 100 µm and a BET specific surface area of from 2 to 200 m²/g_{.}

5. A process according to any one of claims 1 to 4, wherein the inorganic salt is an alkali halide or sulfate, or an earth alkali halide or sulfate.

6. A process according to any one of claims 1 to 5, wherein the inorganic salt is sodium chloride, sodium sulfate or calcium chloride.

7. A process according to any one of claims 1 to 6, wherein the inorganic salt is sodium sulfate or calcium chloride.

8. A process according to any one of claims 1 to 7, wherein the ratio by weight of inorganic salts to urea-formaldehyde resin is 1:500 to 1:1.

9. A process according to any one of claims 1 to 8, wherein the urea-formaldehyde/fluorescent whitening agent suspension is subsequently treated with an emulsion of long-chain alcohols or derivatives thereof, of derivatives of ethylene oxide-alcohols, of paraffin waxes, or of hydrogenated natural or synthetic resins.

10. A process according to any one of claims 1 to 9, wherein the brightener pigment is isolated by filtration and no separate drying or milling step is carried out.

11. A process according to any one of claims 1 to 10, wherein there is used a fluorescent whitening agent of formula in which formulae
each R₁ is independently from each other a radical of formula -NH₂; -O-C₁-C₄alkyl; -O-aryl; -NH-C₁-C₄alkyl; -N(C₁-C₄alkyl)₂; -N(C₁-C₄alkyl)(C₁-C₄hydroxyalkyl); -N(C₁-C₄hydroxyalkyl)₂; -NH-aryl; morpholino or -S-C₁-C₄alkyl(aryl);
each R₂ is independently from each other hydrogen; an unsubstituted or substituted alkyl or aryl group; a radical of formula -OH; -NH₂; -N(CH₂CH₂OH)₂;
R₃ -N[CH₂CH(OH)CH₃]₂; -NH-R₄; -N(R₄)₂; -OR₄; -Cl; , -O-C₁-C₄alkyl; -O-aryl; -NH-C₁-C₄alkyl; -N(C₁-C₄alkyl)₂; -N(C₁-C₄alkyl)(C₁-C₄hydroxyalkyl); -N(C₁-C₄hydroxyalkyl)₂; -NH-aryl, or -S-C₁-C₄alkyl(aryl); is an unsubstituted or substituted alkyl or aryl group;
each R₄ is independently from each other M, or an unsubstituted or substituted alkyl or aryl group;
R₅ is hydrogen; an unsubstituted or substituted alkyl or aryl group; or -NR₇R₈, wherein R₇ and R₈ are each independently of the other hydrogen or an unsubstituted or substituted alkyl or aryl group, or R₇ and R₈ together with the nitrogen atom linking them form a heterocyclic radical, especially a morpholino or piperidino radical;
F₆ is hydrogen, or an unsubstituted or substituted alkyl or aryl group;
R₉ and R₁₀ are each independently of the other hydrogen, C₁-C₄alkyl, phenyl or a radical of formula
R₁₁ is hydrogen, -Cl or SO₃M;
each R₁₂ is independently from each other -CN; -SO₃M; -S(C₁-C₄alkyl)₂ or -S(aryl)₂;
each R₁₃ is independently from each other hydrogen; -SO₃M; -O-C₁-C₄alkyl; -CN; -Cl; COO-C₁-C₄alkyl or -CON(C₁-C₄alkyl)₂;
each R₁₄ is independently from each other hydrogen; -C₁-C₄alkyl; -Cl or -SO₃M;
R₁₅ and R₁₆ are each independently of the other hydrogen, C₁-C₄alkyl; -SO₃M; -Cl or -O-C₁-C₄alkyl;
each R₁₇ is independently of the other hydrogen or C₁-C₄alkyl;
R₁₈ is hydrogen, C₁-C₄alkyl; -CN; -Cl; -COO-C₁-C₄alkyl; -CON(C₁-C₄alkyl)₂; aryl or -O-aryl;
B is
M is hydrogen; sodium; potassium; calcium; magnesium; ammonium; mono-, di-, tri- or tetra-C₁-C₄alkylammonium; mono-, di- or tri-C₁-C₄hydroxyalkylammonium; or ammonium di- or tri-substituted by a mixture of C₁-C₄alkyl and C₁-C₄hydroxyalkyl groups; and
n₁, n₂ and n₃ are each independently of the others 0 or 1.

12. A process according to claim 11, wherein a fluorescent whitening agent of formula (4) is used.

13. An additive in the form of a brightener pigment comprising
a) a water-insoluble urea-formaldehyde resin having a water content of more than or equal to 50% by weight, and
(b) a water-soluble fluorescent whitening agent.

## Patentansprüche

1. Verfahren zur Herstellung eines Aufhellungspigments, umfassend
(a) ein in Wasser unlösliches Harnstoff-Formaldehyd-Harz mit einem Wassergehalt von mehr als oder gleich 50 Gewichtsprozent, und
(b) ein in Wasser lösliches fluoreszierendes Weißungsmittel,
wobei das Verfahren umfasst
Zusammen-Geben von (a), (b) und einem anorganischen Salz, wobei die Menge des anorganischen Salzes ausreichend ist, um Abscheidung des in Wasser löslichen fluoreszierenden Weißungsmittels (b) auf dem in Wasser unlöslichen Harnstoff-Formaldehyd-Harz (a) zu bewirken.

2. Verfahren nach Anspruch 1, wobei der Wassergehalt von dem in Wasser unlöslichen Harnstoff-Formaldehyd-Harz 50 bis 90 Gewichtsprozent ist.

3. Verfahren nach Anspruch 1, wobei der Wassergehalt von dem in Wasser unlöslichen Harnstoff-Formaldehyd-Harz 60 bis 90 Gewichtsprozent ist.

4. Verfahren nach einem der Ansprüche 1 bis 3, wobei das in Wasser unlösliche Harnstoff-Formaldehyd-Harz ein Molverhältnis von Harnstoff zu Formaldehyd von 1 : 1,3 bis 2 Mol, einen Teilchendurchmesser von 0,01 bis 100 µm und eine spezifische BET-Oberfläche von 2 bis 200 m²/g aufweist.

5. Verfahren nach einem der Ansprüche 1 bis 4, wobei das anorganische Salz ein Alkalihalogenid oder -sulfat oder ein Erdalkalihalogenid oder -sulfat ist.

6. Verfahren nach einem der Ansprüche 1 bis 5, wobei das anorganische Salz Natriumchlorid, Natriumsulfat oder Calciumchlorid ist.

7. Verfahren nach einem der Ansprüche 1 bis 6, wobei das anorganische Salz Natriumsulfat oder Calciumchlorid ist.

8. Verfahren nach einem der Ansprüche 1 bis 7, wobei das Gewichtsverhältnis von anorganischen Salzen zu Harnstoff-Formaldehyd-Harz 1 : 500 bis 1 : 1 ist.

9. Verfahren nach einem der Ansprüche 1 bis 8, wobei die Harnstoff-Formaldehyd / fluoreszierendes Weißungsmittel-Suspension anschließend mit einer Emulsion von langkettigen Alkoholen oder Derivaten davon, von Derivaten von Ethylenoxid-Alkoholen, von Paraffinwachsen, oder von hydrierten natürlichen oder synthetischen Harzen behandelt wird.

10. Verfahren nach einem der Ansprüche 1 bis 9, wobei das Aufhellungspigment durch Filtration isoliert wird und kein separater Trocknungs- oder Vermahlungsschritt ausgeführt wird.

11. Verfahren nach einem der Ansprüche 1 bis 10, wobei ein fluoreszierendes Weißungsmittel der Formel verwendet wird,
wobei in den Formeln
jedes R₁ unabhängig voneinander einen Rest der Formel -NH₂; -O-C₁-C₄-Alkyl; -O-Aryl; -NH-C₁-C₄-Alkyl; -N(C₁-C₄-Alkyl)₂; -N(C₁-C₄-Alkyl)(C₁-C₄-hydroxyalkyl); -N(C₁-C₄-Hydroxyalkyl)₂; -NH-Aryl; Morpholino oder -S-C₁-C₄-Alkyl(aryl) darstellt;
jedes R₂ unabhängig voneinander Wasserstoff; eine unsubstituierte oder substituierte Alkyl- oder Aryl-Gruppe; einen Rest der Formel -OH; -NH₂; -N(CH₂CH₂OH₎₂; -N[CH₂CH(OH)CH₃]₂; -NH-R₄; -N(R₄)₂; -OR₄; -Cl; -O-C₁-C₄-Alkyl; -O-Aryl; -NH-C₁-C₄-Alkyl; -N(C₁-C₄-Alkyl)₂; -N(C₁-C₄-Alkyl)(C₁-C₄-hydroxyalkyl); -N(C₁-C₄-Hydroxyalkyl)₂; -NH-Aryl oder -S-C₁-C₄-Alkyl(aryl) darstellt;
R₃ eine unsubstituierte oder substituierte Alkyl- oder Aryl-Gruppe darstellt;
jedes R₄ unabhängig voneinander M oder eine unsubstituierte oder substituierte Alkyl- oder Aryl-Gruppe darstellt; R₅ Wasserstoff; eine unsubstituierte oder substituierte Alkyl- oder Aryl-Gruppe; oder -NR₇R₈, worin R₇ und R₈ jeweils unabhängig voneinander Wasserstoff oder eine unsubstituierte oder substituierte Alkyl- oder Aryl-Gruppe darstellen, oder R₇ und R₈, zusammen mit dem Stickstoffatom, das sie verbindet, einen heterocyclischen Rest, insbesondere einen Morpholino- oder Piperidino-Rest, bilden, darstellt;
R₆ Wasserstoff oder eine unsubstituierte oder substituierte Alkyl- oder Aryl-Gruppe darstellt;
R₉ und M₁₀ jeweils unabhängig voneinander Wasserstoff, C₁-C₄-Alkyl, Phenyl oder einen Rest der Formel darstellen; R₁₁ Wasserstoff, -Cl oder SO₃M darstellt;
jedes R₁₂ unabhängig voneinander -CN; -SO₃M; -S(C₁-C₄-Alkyl)₂ oder -S(Aryl)₂ darstellt;
jedes R₁₃ unabhängig voneinander Wasserstoff; -SO₃M; -O-C₁-C₄-Alkyl; -CN; -Cl; COO-C₁-C₄-Alkyl oder -CON(C₁-C₄-Alkyl)₂ darstellt;
jedes R₁₄ unabhängig voneinander Wasserstoff; -C₁-C₄-Alkyl; -Cl oder -SO₃M darstellt;
R₁₅ und R₁₆ jeweils unabhängig voneinander Wasserstoff, C₁-C₄-Alkyl; -SO₃M; -Cl oder -O-C₁-C₄-Alkyl darstellen;
jedes R₁₇ unabhängig voneinander Wasserstoff oder C₁-C₄-Alkyl darstellt;
R₁₈ Wasserstoff, C₁-C₄-Alkyl; -CN; -Cl; -COO-C₁-C₄-Alkyl; -CON(C₁-C₄-Alkyl)₂; Aryl oder -O-Aryl darstellt;
B darstellt;
M Wasserstoff; Natrium; Kalium; Calcium; Magnesium; Ammonium; Mono-, Di-, Tri- oder Tetra-C₁-C₄-alkylammonium; Mono-, Di- oder Tri-C₁-C₄-hydroxyalkylammonium; oder Ammonium, di- oder tri-substituiert mit einem Gemisch von C₁-C₄-Alkyl- und C₁-C₄-Hydroxyalkyl-Gruppen, darstellt; und
n₁, n₂ und n₃ jeweils unabhängig voneinander 0 oder 1 sind.

12. Verfahren nach Anspruch 11, wobei das fluoreszierende Weißungsmittel der Formel (4) verwendet wird.

13. Additiv in Form eines Aufhellungspigments, umfassend
(a) ein in Wasser unlösliches Harnstoff-Formaldehyd-Harz mit einem Wassergehalt von mehr als oder gleich 50 Gewichtsprozent und
(b) ein in Wasser lösliches fluoreszierendes Weißungsmittel.

## Revendications

1. Procédé de préparation d'un pigment optique de type azurant comprenant
(a) une résine urée-formaldéhyde insoluble dans l'eau ayant une teneur en eau supérieure ou égale à 50 % en poids, et
(b) un agent de blanchiment fluorescent soluble dans l'eau,
lequel procédé comprend l'étape consistant à
mélanger (a), (b) et un sel inorganique, la quantité du sel inorganique étant suffisante pour effectuer un dépôt de l'agent de blanchiment fluorescent soluble dans l'eau (b) sur la résine urée-formaldéhyde insoluble dans l'eau (a).

2. Procédé selon la revendication 1, dans lequel la teneur en eau de la résine urée-formaldéhyde insoluble dans l'eau est de 50 à 90 % en poids.

3. Procédé selon la revendication 1, dans lequel la teneur en eau de la résine urée-formaldéhyde insoluble dans l'eau est de 60 à 90 % en poids.

4. Procédé selon l'une quelconque des revendications 1 à 3, dans lequel la résine urée-formaldéhyde insoluble dans l'eau a un rapport molaire urée sur formaldéhyde de 1 : 1,3 à 2 moles, un diamètre de particule de 0,01 à 100 µm et une surface spécifique BET de 2 à 200 m²/g.

5. Procédé selon l'une quelconque des revendications 1 à 4, dans lequel le sel inorganique est un halogénure ou un sulfate alcalin, ou un halogénure ou un sulfate alcalino-terreux.

6. Procédé selon l'une quelconque des revendications 1 à 5, dans lequel le sel inorganique est le chlorure de sodium, le sulfate de sodium ou le chlorure de calcium.

7. Procédé selon l'une quelconque des revendications 1 à 6, dans lequel le sel inorganique est le sulfate de sodium ou le chlorure de calcium.

8. Procédé selon l'une quelconque des revendications 1 à 7, dans lequel le rapport en poids des sels inorganiques sur la résine urée-formaldéhyde est de 1 : 500 à 1 : 1.

9. Procédé selon l'une quelconque des revendications 1 à 8, dans lequel la suspension urée-formaldéhyde / agent de blanchiment fluorescent est traitée ultérieurement avec une émulsion d'alcools à longue chaîne ou de dérivés de ceux-ci, de dérivés d'oxyde d'éthylène-alcools, de cires de paraffine, ou de résines naturelles ou synthétiques hydrogénées.

10. Procédé selon l'une quelconque des revendications 1 à 9, dans lequel le pigment de type azurant optique est isolé par filtration et aucune étape de séchage ou de broyage séparée n'est réalisée.

11. Procédé selon l'une quelconque des revendications 1 à 10, dans lequel on utilise un agent de blanchiment fluorescent de formule dans lesquelles formules
chaque R₁ est indépendamment des autres un radical de formule -NH₂ ; -O-alkyle en C₁ à C₄ ; -O-aryle ; -NH-alkyle en C₁ à C₄ ; -N(alkyle en C₁ à C₄)₂ ;
-N(alkyl en C₁ à C₄)(hydroxyalkyle en C₁ à C₄) ; -N(hydroxyalkyle en C₁ à C₄)₂ ; -NH-aryle ; morpholino ou -S-alkyl en C₁ à C₄(aryle) ;
chaque R₂ est indépendamment des autres un atome d'hydrogène ; un groupe alkyle ou aryle non substitué ou substitué ; un radical de formule -OH ; -NH₂ ; -N(CH₂CH₂OH)₂ ; -N[CH₂CH(OH)CH₃]₂ ; -NH-R₄ ; -N(R₄)₂ ; - OR₄ ; -Cl ; -O-alkyle en C₁ à C₄ ; -O-aryle ; -NH-alkyle en C₁ à C₄ ; -N-(alkyle en C₁ à C₄)₂ ; -N(alkyl en C₁ à C₄)(hydroxyalkyle en C₁ à C₄) ; -N(hydroxyalkyle en C₁ à C₄)₂ ; -NH-aryle ; ou -S-alkyl en C₁ à C₄(aryle) ;
R₃ est un groupe alkyle ou aryle non substitué ou substitué ;
chaque R₄ est indépendamment des autres M, ou un groupe alkyle ou aryle non substitué ou substitué ;
R₅ est un atome d'hydrogène ; un groupe alkyle ou aryle non substitué ou substitué ; ou -NR₇R₈, où R₇ et R₈ sont chacun indépendamment l'un de l'autre un atome d'hydrogène ou un groupe alkyle ou aryle non substitué ou substitué, ou bien R₇ et R₈ conjointement avec l'atome d'azote les liant forment un radical hétérocyclique, spécialement un radical morpholino ou pipéridino ;
R₆ est un atome d'hydrogène, ou un groupe alkyle ou aryle non substitué ou substitué ;
R₉ et R₁₀ sont chacun indépendamment l'un de l'autre un atome d'hydrogène, un groupe alkyle en C₁ à C₄, phényle ou un radical de formule R₁₁ est un atome d'hydrogène, -Cl ou SO₃M ;
chaque R₁₂ est indépendamment des autres -CN ; -SO₃M ; -S(alkyle en C₁ à C₄)₂ ou -S(aryle)₂ ;
chaque R₁₃ est indépendamment des autres un atome d'hydrogène, un groupe - SO₃M ; -O-alkyle en C₁ à C₄ ; -CN ; -Cl ; COO-alkyle en C₁ à C₄ ou -CON(alkyle en C₁ à C₄)₂ ;
chaque R₁₄ est indépendamment des autres un atome d'hydrogène, un groupe alkyle en C₁ à C₄ ; -Cl ou -SO₃M ;
R₁₅ et R₁₆ sont indépendamment l'un de l'autre un atome d'hydrogène, un groupe alkyle en C₁ à C₄ ; -SO₃M ; -Cl ou -O-alkyle en C₁ à C₄ ;
chaque R₁₇ est indépendamment des autres un atome d'hydrogène ou un groupe alkyle en C₁ à C₄ ;
R₁₈ est un atome d'hydrogène, un groupe alkyle en C₁ à C₄ ; -CN ; -Cl ; -COO-alkyle en C₁ à C₄ ou -CON(alkyle en C₁ à C₄)₂ ; aryle ou -O-aryle ; B est M est un atome d'hydrogène ; de sodium ; de potassium ; de calcium ; de magnésium ; un groupe ammonium ; mono-, di-, tri- ou tétra-alkyl(en C₁ à C₄)ammonium ; mono-, di- ou trihydroxyalkyl(en C₁ à C₄)ammonium ; ou ammonium di- ou tri-substitué par un mélange de groupes alkyle en C₁ à C₄ et hydroxyalkyle en C₁ à C₄ ; et
n₁, n₂ et n₃ valent chacun indépendamment des autres 0 ou 1.

12. Procédé selon la revendication 11, dans lequel un agent de blanchiment fluorescent de formule (4) est utilisé.

13. Additif sous la forme d'un pigment optique de type azurant comprenant
(a) une résine urée-formaldéhyde insoluble dans l'eau ayant une teneur en eau supérieure ou égale à 50 % en poids, et
(b) un agent de blanchiment fluorescent soluble dans l'eau.
